

Aug. 16, 1955

G. MEISTER

2,715,691

VAPOR DISCHARGE LAMP

Filed June 29, 1951

Fig. 1.



Fig. 2.



Fig. 3.



INVENTOR  
GEORGE MEISTER.

BY *Dr. J. Kelly*  
ATTORNEY

## 1

2,715,691

## VAPOR DISCHARGE LAMP

George Meister, Newark, N. J., assignor to Westinghouse Electric Corporation, East Pittsburgh, Pa., a corporation of Pennsylvania

Application June 29, 1951, Serial No. 234,395

1 Claim. (Cl. 313—25)

This invention relates to lamps and, more particularly, to improved metal vapor discharge lamps.

In metal vapor discharge lamps, particularly those containing alkali metals, which operate at relatively high temperatures, that is, above 200° C., the making of metal glass seals which are impervious to attack by the vaporized metal has presented a real problem. The metal glass seals in such tubes usually consist of a refractory metal leading-in conductor, suitably tungsten, and have an oxide layer at the metal-glass interface. This oxide layer fails to withstand the attack of the reducing metal vapor, such as cesium vapor, at about 200° C.

Some improvement has been obtained through the use of molybdenum leading-in conductors in lamps which operate up to approximately 250° C. However, even these molybdenum glass seals fail above 280° C. when the cesium vapor attains sufficient pressure to force its way into contact with the protective intermediate layer of oxide in the metal glass seal, thereby combining with the oxygen of said layer to form, in the case of cesium, cesium oxide within the tube and to produce a leakage path along the leading-in conductors.

Hence, it has been found advantageous, according to my invention, to make the metal-glass seal in alkali metal vapor lamps, such as cesium, with a degasified borosilicate glass and a refractory metal leading-in conductor which remains metallic and has no intermediate oxide layer at the interface between the glass and the said conductors which the cesium vapor can attack. During the sealing of said conductor to said degasified borosilicate glass, I prevent the formation of the intermediate oxide layer on the glass metal interface by holding the refractory metal leading-in conductor in or at the tip of the reducing part of an oxy-hydrogen flame so that no oxide can form or, if such an oxide is formed, it is immediately vaporized from the conductor by the hot flame.

In its general aspect, the present invention has the object of overcoming the aforementioned disadvantages of the prior art in metal vapor discharge tubes.

Specifically, an object of the present invention is an alkali metal vapor lamp having a seal between a refractory metal leading-in conductor and a degasified borosilicate glass which will withstand action by said metal vapor.

Another and specific object is an alkali metal vapor lamp having a seal between a refractory metal leading-in conductor and a degasified borosilicate glass without formation of an intermediate oxide layer at the glass interface.

An additional object is a method of sealing a refractory metal leading-in conductor to a degasified borosilicate glass of an alkali metal vapor lamp comprising heating said conductor in or at the tip of the reducing part of an oxy-hydrogen flame so that no oxide forms at the glass metal interface, or if said oxide is formed thereat, it is immediately vaporized by the hot flame during the sealing of said conductor to said glass.

Another object of the invention is a metal vapor lamp

## 2

operating at temperatures at which said metal vapor will reduce any oxide of refractory metal used in effecting a seal and having a seal between a refractory metal leading-in conductor and a degasified borosilicate glass which is impervious to reduction by the metal vapor and resultant early life leakage failures through the seal along the conductor.

Other objects and advantages will appear to those skilled in the art to which it appertains as the description thereof proceeds, both by direct recitation thereof, and by implication from the context.

Referring to the accompanying drawing, in which like numerals of reference indicate similar parts throughout:

Fig. 1 is an elevational view of a metal vapor lamp embodying my invention;

Fig. 2 is an enlarged fragmentary axial sectional view of one end of the lamp of Fig. 1;

Fig. 3 is an elevational view of a seal between a refractory leading-in conductor of the lamp of Fig. 1 and a degasified borosilicate glass bead.

Referring to the drawing in detail, the reference numeral 10 designates an alkali metal vapor lamp comprising an inner envelope or arc tube 12, an outer evacuated envelope 14 desirably enclosing a gettering device 16, and oppositely disposed electrode mounts 18 and 20.

The generally cylindrical arc tube 12 is desirably of alkali-resistant vitreous material, such as glass No. 1, a soda-aluminum borosilicate glass with a small percentage of alumina, and is desirably coated on its interior with a glaze composed largely of boric oxide. This glass is designated as a tungsten sealing glass. It has a softening point at 703° C., an annealing point of 496° C., a strain point of 461° C., a coefficient of expansion of  $46 \times 10^{-7}$  between 0 and 300° C., and a density of 2.23. The log<sub>10</sub> of its resistivity at 350° C. is 6.77. Its power factor is .0033 (expressed as a decimal and not as percent), its dielectric constant 4.9 and its loss factor .0161 (expressed as a decimal and not as percent). This glass has the following approximate composition:

|                                            | Per cent |
|--------------------------------------------|----------|
| SiO <sub>2</sub> -----                     | 67       |
| B <sub>2</sub> O <sub>3</sub> -----        | 22       |
| Al <sub>2</sub> O <sub>3</sub> -----       | 2½       |
| Na <sub>2</sub> O + K <sub>2</sub> O ----- | 7        |
| Miscellaneous -----                        | 1½       |

This tube 12 contains an inert gaseous filling, such as argon at about 20 cm. pressure, for initiating and sustaining a discharge, and a small quantity of a metal, such as cesium, which is readily vaporizable. While a cesium vapor lamp has been selected as an embodiment of this invention, it will be understood that other alkali metal vapor lamps or vapor lamps employing metals which readily reduce refractory metal oxides at their operating temperatures are contemplated. To each end of tube 12 is attached a hollow extension 22 of reduced diameter. To these extensions are axially sealed, as hereinafter explained, refractory leading-in conductors 23 of electrode mounts 18 and 20.

The electrode mount 18 comprises a filamentary electrode 24 having an oxide coated helix 25 surrounding a straight return portion 26. It is secured to the inner extremities of conductors 23 as by welding. Near the outer portion of one conductor 23 is the gettering means 16 mounted by means of a connector 27 in close proximity to the outer bulb 14. The outer ends of conductors 23 are connected by flexible, desirably semi-circular connectors 28 to outer leads 30, which in turn are sealed through a stem 31 to the outer envelope 14.

The electrode mount 20 differs from mount 18 only in the addition of a cup-like anode 32 surrounding the electrode 24 and electrically joined by connector 34 to

one of the leading-in conductors 23. This anode is employed for direct current operation of the lamp 10. The outer extremities of conductors 23 of mount 20 are joined by flexible connectors 34 to outer leads 36. The leads 36 in turn are secured, as by welding, to hollow cup-like outer pins 37. These pins 37 are sealed to dish-like projections 35 at one end of the envelope 14.

About each of the above-mentioned extensions 22 of arc tube 12 are two suitable resilient supporting collars 38, each having a semi-circular body 39 clamped to each other and about the extensions 22 by bolts and nuts, and spring arm extensions 40 projecting outwardly perpendicular from the plane of the body 39 to the inner wall of outer envelope 14. A heat resistant tape, such as glass tape, is desirably employed between said collars 38 and the extensions 22.

In outer vitreous envelope 14, employed for conserving the heat of operation, there is provided an exhaust tubulation 41 for evacuation purposes. A suitable base 42 is affixed at the end opposite pins 37 for making a connection to the outer leads 30 of mount 18.

According to my invention, the metal vapor lamp 10 is provided with an oxide-free seal which the metal vapor will not spoil at operating temperatures above 300° C., that is, between 307° and 325° C., between the leading-in conductors 23 of electrode mounts 18 and 20 and the extensions 22 of arc tube 12. This approximately 300° C. operating temperature corresponds to 2 watts input per cm.<sup>-2</sup> of the surface of arc tube 12 when the lamp is operated within an outer envelope 14.

First, the refractory leading-in conductors 23, suitably tungsten or molybdenum, are chemically cleaned electrolytically to remove any oxide thereon and produce a clean, bright, metallic surface. The clean conductors 23 are then heated in or at the tip or inner cone of an oxy-hydrogen flame and hermetically sealed to or coated with a bead 44 of a degasified borosilicate glass, such as glass No. 2, as shown in Fig. 3.

This glass No. 2, a soda aluminum borosilicate glass, is designated H. R. Clear Chemical. It has a softening point at  $820 \pm 1 \times 10^{-7}$  between 0 and 300° C., an approximate working point of 1220° C. and a density of 2.23. The  $\log_{10}$  of its resistivity at 350° C. is 6.68. Its power factor is .0046 (expressed as a decimal and not as percent); its dielectric constant 4.6 and its loss factor .021 (expressed as a decimal and not as percent).

This glass has the following approximate composition:

|                                      | Per cent |
|--------------------------------------|----------|
| SiO <sub>2</sub>                     | 80       |
| B <sub>2</sub> O <sub>3</sub>        | 13       |
| Al <sub>2</sub> O <sub>3</sub>       | 2        |
| Na <sub>2</sub> O + K <sub>2</sub> O | 4½       |
| Miscellaneous                        | ½        |

The degasified borosilicate glass No. 2 is obtained by heating said glass to a temperature of about 1700° C. to remove the gases therefrom. The intermediate oxide layer which normally forms at the metal glass interface, is avoided by the use of the degasified borosilicate glass, and the reducing action of the oxy-hydrogen sealing flame, which prevents formation of the refractory metal oxide on conductors 23, or if the oxide is formed thereon, immediately vaporizes said oxide from said conductors.

Employing a suitable jig (not shown) affixed to one end of conductors 23 the filamentary electrode 24 is mounted on the opposite extremities of conductors 23. These conductors 23, still aligned in the fixture, are sealed together at the beads 44 by a button 46 of degasified borosilicate glass, such as glass No. 2, the same glass employed for the beads 44.

The mount 18, so formed, is in turn sealed by means of the button 46 to the extension 22 of arc tube 12. In

like manner, the mount 20 is sealed to the oppositely disposed extension 22 of arc tube 12.

After a suitable exhaust, which may consist of a bake, filamentary electrode treatment, evacuation and final gas and metal fill, the arc tube 12 is tipped off as at 47. The oppositely disposed electrode mounts 18 and 20 are joined by connectors 28 and 34 to the outer leads 30 and 36 respectively. The support collars 38 are secured about extensions 22 of arc tube 12, and the outer envelope 14 is aligned about tube 12 by means of extensions 40 of collars 38. After the upper end of outer envelope 14 is flared inwardly, the stem 31 is sealed thereto. Outer leads 36 are secured to the outer pins 37 which are then sealed to the projections 35 on the opposite end of envelope 14. After a suitable exhaust, desirably consisting of a bake and evacuation through tubulation 41, the envelope 14 is tipped off. The gettering means 16 is vaporized on to the interior wall of envelope 14 and a base 42 is applied, thereby completing the lamp 10.

Thus it will be seen from the foregoing description that I have constructed a metal vapor lamp 10 having a seal between refractory metal leading-in conductors 23 and a degasified borosilicate glass bead 44 which will withstand metal vapor at operating temperatures of the lamp where said metal vapor normally would reduce any oxide of a refractory metal conductor. This seal between the refractory metal leading-in conductors 23 and the degasified borosilicate glass bead 44 is made without the formation of an intermediate oxide layer at the metal-glass interface. In addition, the above-mentioned seal being impervious to the metal vapor at the operating temperatures in the lamp 10, a resultant early leakage failure through the seal along said conductors 23 are eliminated, as well as seals cracked from overheating.

Although a preferred embodiment of my invention has been disclosed, it will be understood that modifications may be made within the spirit and scope of the appended claim.

I claim:

A cesium vapor lamp adapted to operate at about 2 watts per square centimeter of the inner envelope surface area to maintain said cesium as a vapor at a temperature at about 300° C. and comprising an inner vitreous light transmitting envelope, oppositely disposed electrode mounts in said inner envelope and each having at least two tungsten leading-in conductors and a filamentary electrode thereon, an hermetic seal between said conductors and said inner envelope, with said conductors being oxide-free at least along substantially the length of said hermetic seal thereon, said seal having degasified borosilicate glass hermetically fused directly to said oxide-free tungsten conductors without an oxide bond at the metal-glass interface and through a degasified borosilicate glass button to said inner envelope, an ionizable medium in said inner envelope for initiating and sustaining a discharge admixed with small quantity of cesium which is readily vaporizable and an outer evacuated vitreous light transmitting envelope enclosing said inner envelope for conserving the heat of operation.

#### References Cited in the file of this patent

#### UNITED STATES PATENTS

|           |          |                |
|-----------|----------|----------------|
| 1,984,426 | Pirani   | Dec. 18, 1934  |
| 1,990,205 | Reger    | Feb. 5, 1935   |
| 2,060,610 | Cox      | Nov. 10, 1936  |
| 2,068,596 | Cox      | Jan. 19, 1937  |
| 2,228,327 | Spanner  | Jan. 14, 1941  |
| 2,330,072 | Meister  | Sept. 21, 1943 |
| 2,504,521 | Greiner  | Apr. 18, 1950  |
| 2,617,068 | Spinnler | Nov. 4, 1952   |